

N. BENDIXEN.

METHOD OF PRODUCING PAPER MATRICES FOR HALF-TONE STEREOTYPING.

APPLICATION FILED NOV. 9, 1911.

1,108,677.

Patented Aug. 25, 1914.

Fig. 1.



Fig. 2.



Fig. 3.



Fig. 4.



Witnesses;  
J. M. Myntkoop,  
Sanford Deerington.

Inventor,  
Nels Bendixen,  
By Kingshott Bros  
Attorneys.

# UNITED STATES PATENT OFFICE.

NIELS BENDIXEN, OF COPENHAGEN, DENMARK.

## METHOD OF PRODUCING PAPER MATRICES FOR HALF-TONE STEREOTYPING.

1,108,677.

Specification of Letters Patent. Patented Aug. 25, 1914.

Application filed November 9, 1911. Serial No. 659,415.

To all whom it may concern:

Be it known that I, NIELS BENDIXEN, subject of the King of Denmark, residing at Studiestræde 28, Copenhagen, Denmark, 5 have invented new and useful Improvements in Methods of Producing Paper Matrices for Half-Tone Stereotyping, of which the following is a specification.

The invention relates to a method of producing paste-covered paper matrices for the stereotyping of half-tone printing blocks, and the object of the invention is to make it possible to produce such matrices very quickly and to render them impervious to 15 the humidity of the atmosphere whereby they become easily mailable.

The extremely rapid evolution of the illustrated press and the great demands made upon it have made it necessary to procure the illustrated matter with extreme rapidity, while at the same time the demand for steady increase in the amount of illustrated matter has made it a very important problem to effect a reduction of the cost of 20 making the blocks. At the present state of the art of illustration, when an event is to be illustrated in the world's press this is done by mailing, from the locality concerned, photographs of the event, often by the hundred, to the illustrated press all over the 25 world. At every place where these photographs are received etchings, and often quite expensive ones, are produced therefrom, and the total cost of production of these many 30 etchings run into considerable sums, and besides much time is wasted by the exactly identical process, namely the etching, being repeated at so many different places.

The present invention has for its object 35 partly to save money, partly to save time for the illustrated press, and it is carried into effect in the following manner:

In the accompanying drawing illustrating the different steps in carrying out this 40 method, Figure 1 shows a section through the etching *a*; Fig. 2 a similar view to Fig. 1 with a coat of paste *b* applied; Fig. 3 shows the next step, when the paper floss *c* has been laid upon the paste coated etching of 45 Fig. 2; and Fig. 4 shows the completed paper matrix removed from the etching.

From a photograph an etching *a* is made. This is coated by an especially prepared paste *b* constituting a part of this invention. 50 By means of another special paste, being also an integral part of the invention, a

moist matrix backing *c* is made, *i. e.* one pasted together of layers of tissue paper and so-called plate paper, that means the kind of paper used in copper plate printing; 55 this matrix is placed on top of the coated etching, covered by blotting paper and placed in a heated drying press. The coating on the etching will then loosen itself from the etching and adhere to the paper 60 matrix, transferring to the paper all the details of the etching. In this manner a paper floss is procured, which is flexible and adapted to be sent by mail and wherein, immediately after its production, one or 65 several castings may be made, using a suitable metal alloy, the so called stereotype metal.

Such paper matrices containing the details of the etching may be produced in very 70 few minutes, owing to the special composition of the matrix paste, and very much quicker than a photograph might be produced, and as an unlimited number of matrices may be produced from the same one 75 etching, and the receivers of these, at a very insignificant cost may "stereotype" a printing block on the paper matrix received, and may, after having used the block for printing, remelt it and use it for a new block, this 80 invention means, in practice, a very extraordinary saving of time and money, because only one etching of the event has to be made, because the paper matrices may be produced at a minimum cost, because the receiver of 85 the paper matrix avoids the expense of producing an etching, and finally because the receiver of the paper matrix may at once 90 cast a block therein and has not to waste time by producing an etching.

The special features of the invention are 95 the following: For coating the etching a paste is used containing a fatty substance as well as a grease absorbing substance. The fatty substance is contained in the paste in 100 shape of an especially fine emulsion of for instance a paraffin, and is produced by preparing a strong solution of glue, preferably fish glue wherein the paraffin is melted. In preparing this first paste, I preferably use a 105 filling and adhesive substance, an emulsion of a fatty substance, such as an emulsion of paraffin in fish glue and a grease absorbing substance, such as pipe clay. The glue has the peculiar property to dissolve the paraffin 110 into a microscopically fine state without depositing it again, which cannot be attained

in any other of the known manners, for instance not by dissolving the paraffin in a solvent and mixing the solution with the other solid components of the paste. A 5 paste prepared in this manner would prove unfit for use. To the fatty solution of glue prepared, a grease absorbing substance is added, for instance a clayey substance such as pipe-clay. When this paste is spread on 10 the etching, the matrix material is placed thereon, as mentioned above.

The distinguishing feature of this matrix is that it possesses an extraordinary power 15 to dry quickly, absorbing at the same time the fatty substance of the paste. It has been tried to produce quickly drying paper matrices by means of easily volatile fluids, for instance alcohol, but this method has had the draw-back that the alcohol of the damp 20 matrix evaporated too soon, and consequently the matrix became dry, before it entered into the drying press whereby it lost its binding power and instead of forming a solid coherent mass it was loose and liable 25 to be separated sheet for sheet. This draw-back is avoided, according to the present invention, by binding the alcohol by the addition of soap, which will retain the alcohol, even at the temperature to be found in a 30 heated stereotype room, but it will nevertheless allow a quick evaporation of the alcohol, as soon as the etching and the matrix are brought into the heated drying press. The second paste is therefore preferably 35 prepared from an alcoholic solution of soap, a grease absorbing clayey substance and an adhesive, produced by the concoction of dextrin and starch.

The coöperation between the paste coating 40 of the etching and the damp matrix is effected in the drying press in the following manner. When the heat commences to act, the clayey substance of the paste will absorb the admixed fatty substance, and during the 45 continued drying the blotting paper of the matrix as well as its clayey substance will continue this absorption of grease, the result being that the finished picture matrix, throughout its mass, will become fatty, the 50 amount of grease decreasing toward the side which has been nearest to the etching. This is on account of the highly absorbing quality of the porous paper in the flong, which, during the heating absorbs 55 the grease, so that very little of the grease will remain in the paste coating of the matrix. In this manner it has been attained 60 to produce a matrix impervious to the atmospheric humidity and still admitting excellent casting to be made thereon.

Having now particularly described and ascertained the nature of my said invention and in what manner the same is to be performed, I declare that what I claim is:—

65 1. A method of producing a matrix for

stereotyping consisting in first applying to an etching a coating suitable for producing a relief surface; secondly in pasting together several layers of paper to form a pad by means of a paste containing saponaceous, 70 absorbing and adhesive substances; thirdly in placing said pad while damp on said coating; fourthly in pressing said pad upon said coating and lastly in drying the thus produced matrix and subsequently detaching 75 the completed matrix from the etching.

2. A method of producing a paper matrix for stereotyping consisting in first coating a suitable etching with a paste containing adhesive fatty and absorbing substances; secondly in pasting together several layers of paper to form a pad by means of a paste containing saponaceous, absorbing and adhesive substances; thirdly in placing said pad while damp on said coating; fourthly 80 in pressing said pad upon said coating and lastly in drying the thus produced matrix and subsequently detaching the completed matrix 85 from the etching.

3. A method of producing a paper matrix for stereotyping consisting in first coating a suitable etching with a paste containing adhesive, fatty and absorbing substances; secondly in pasting together several layers of paper to form a pad by means of a paste containing saponaceous, absorbing and adhesive substances, said pad being composed of alternate sheets of tissue paper and plate paper; thirdly in placing said pad while damp on said coating; fourthly in pressing said pad upon said coating and lastly in 90 drying the thus produced matrix and subsequently detaching the completed matrix 95 from the etching.

4. A method of producing a paper matrix 105 for stereotyping consisting in first coating a suitable etching with a paste containing adhesive, fatty and absorbing substances; said substances comprising an emulsion of paraffin in fish glue and pipe clay; secondly in 110 pasting together several layers of paper to form a pad by means of a paste containing saponaceous absorbing and adhesive substances; thirdly in placing said pad while damp on said coating; fourthly in pressing 115 said pad upon said coating and lastly in drying the thus produced matrix and subsequently in detaching the completed matrix from the etching.

5. A method of producing a paper matrix 120 for stereotyping consisting in first coating a suitable etching with a paste containing adhesive, fatty and absorbing substances; secondly in pasting together several layers of paper to form a pad by means of a paste 125 containing saponaceous, absorbing and adhesive substances, said substances of the paste being respectively an alcoholic solution of soap, pipe-clay and an adhesive; thirdly in placing said pad while damp on 130

said coating; fourthly in pressing said pad upon said coating and lastly in drying the thus produced matrix and subsequently detaching the completed matrix from the etching.

6. A method of producing a paper matrix for stereotyping consisting in first coating a suitable etching with a paste containing adhesive, fatty and absorbing substances, said 10 substances comprising an emulsion of paraffin in fish glue and pipe clay; secondly in pasting together several layers of paper to form a pad by means of paste containing saponaceous, absorbing and adhesive substances, said pad being composed of alternate sheets of tissue paper and plate-paper,

said substances of the paste being respectively an alcoholic solution of soap, pipe-clay and an adhesive; thirdly in placing said pad while damp on said coating; 20 fourthly in pressing said pad and coating together and lastly in drying the thus produced matrix and subsequently detaching the completed matrix from the etching.

The foregoing specification signed at 25 Copenhagen this 21st day of September, 1911.

NIELS BENDIXEN.

In presence of two witnesses—

JULIUS LEHMANN,  
ORR GIERSING.

Copies of this patent may be obtained for five cents each, by addressing the "Commissioner of Patents, Washington, D. C."